

## UNITED STATES PATENT OFFICE

2,129,840

HEAT-RESISTING OBJECT CONTAINING  
IRON AND ALUMINUMWerner Hessenbruch, Hanau-on-the-Main,  
GermanyNo Drawing. Application September 5, 1936, Se-  
rial No. 99,620. In Germany September 24,  
1935

8 Claims. (Cl. 148—7)

This invention relates to objects made of an alloy containing iron and aluminum.

It is known to make electrical heating elements of alloys which, in addition to iron, contain various amounts of aluminum, for example 2-12% and may also contain chromium in amounts from 0.1 up to about 35%. These alloys are distinguished by the feature that, in general, they are very resistant to heat up to temperatures of about 1,300° C. It is also known that these alloys sometimes exhibit an abnormal phenomenon which may be termed "blistering" (formation of carbuncles). This phenomenon consists in the formation at various places on the heating element for example of black spots, which then lead to accelerated oxidation and to breakage of the heating elements at these places. Reference has been made to this phenomenon for example in the periodical "Elektrowärme," January 1935, in an article entitled "Ueber hochhitzebeständige Chrom-Aluminium-Eisenlegierungen."

According to the present invention, the formation of these blisters or carbuncles and therefore premature local destruction of the heating elements is avoided by treating the material with an alkaline solution before it is brought into operation. For example, the heating elements are placed in a sodium carbonate solution, in lime water, baryta water or caustic soda solution. The duration of the immersion in the alkaline solution may amount, for example, to a few hours but may also be extended to several days.

If the material is then removed from the alkaline solution and the residues of the alkaline constituents are burnt in by heating to a temperature of several hundred degrees the aforementioned tendency to form blisters is entirely removed. The burning in of the alkali can be effected either in a separate operation or when the material is heated for use for the first time.

When the alkaline solution employed for the treatment of the material is such that a "skin" consisting of alkaline constituents is formed on the surface of the solution, as occurs for example in the case of lime water, it is then advisable to remove this skin from the solution before the material is removed from the solution in order that the skin may not adhere to the material itself.

I claim:

1. The method of increasing the resistance to heat of objects made of a ferritic alloy containing iron and aluminum which method comprises subjecting the objects to the action of an alkaline solution of the group of sodium carbonate

solution, lime water, baryta water, and caustic soda solution, removing the objects from the alkaline solution and drying in the remaining alkaline constituents.

2. The method of increasing the resistance to heat of objects made of an alloy consisting of iron and aluminum, which method comprises subjecting the objects to the action of an alkaline solution of the group of sodium carbonate solution, lime water, baryta water, and caustic soda solution, removing the objects from the alkaline solution and drying in the remaining alkaline constituents.

3. The method of increasing the resistance of heat of objects made of an alloy consisting of iron, aluminum and chromium, which method comprises subjecting the objects to the action of an alkaline solution of the group of sodium carbonate solution, lime water, baryta water, and caustic soda solution, removing the objects from the alkaline solution and drying in the remaining alkaline constituents.

4. The method of increasing the resistance to heat of objects made of an alloy containing iron and aluminum, which method consists in immersing the objects for a period of from several hours to several days in an alkaline solution of the group of sodium carbonate solution, lime water, baryta water, and caustic soda solution, removing the objects from the alkaline solution and drying in the remaining alkaline constituents.

5. The method of increasing the resistance to heat of objects made of an alloy containing iron and aluminum, which method consists in immersing the objects for a period of from several hours to several days in an alkaline solution of the group of sodium carbonate solution, lime water, baryta water, and caustic soda solution, and removing a deposit formed on the solution before removing the objects from the solution.

6. The method of increasing the resistance to heat of objects made of an alloy consisting of iron, aluminum and chromium which method consists in immersing the objects for a period of from several hours to several days in an alkaline solution of the group of sodium carbonate solution, lime water, baryta water, and caustic soda solution, removing the objects from the alkaline solution and drying in the remaining alkaline constituents.

7. The method of increasing the resistance to heat of objects made of an alloy consisting of iron, aluminum and chromium, which method consists in subjecting the objects to the action

of an alkaline solution of the group of sodium carbonate solution, lime water, baryta water, and caustic soda solution, removing the objects from the alkaline solution, and then subjecting the 5 objects to a temperature of several hundred degrees centigrade.

8. The method of increasing the resistance to heat of objects made of an alloy consisting of iron, aluminum and chromium, which method

consists in immersing the objects for a period of from several hours to several days in an alkaline solution of the group of sodium carbonate solution, lime water, baryta water, and caustic soda solution, removing a deposit formed thereon, removing the objects from the solution, and drying in the remaining alkaline constituents.

WERNER HESSENBRUCH.